

Patented June 3, 1924.

1,496,268

# UNITED STATES PATENT OFFICE.

ANNA SCHWARZ, GEB. HOPPEHEL, OF BERLIN, GERMANY, ASSIGNOR TO AUGUST CARL LENTZ, OF IRON RIDGE, WISCONSIN.

## PHOTOMECHANICAL PROCESS.

No Drawing.

Application filed June 13, 1923. Serial No. 645,198.

To all whom it may concern:

Be it known that I, ANNA SCHWARZ, geb. HOPPEHEL, a citizen of Germany, and a resident of Berlin, Prussia, Germany, have invented new and useful Improvements in Photomechanical Process, of which the following is a full, clear, and exact specification.

My invention relates to photo-mechanical processes and refers particularly to the production of zinc printing plates.

The present employed methods of producing zinc printing plates through the medium of bichromate emulsions, with or without the employment of transfer prints present numerous difficulties and produce plates so far removed from desirable attributes, that their application has been largely replaced by other photo-mechanical methods.

The use of bichromate emulsions upon grained, or rough, zinc plates has in particular many disadvantages, among which is the liability of the bichromate film to break and to become sharp and pointed, thus producing irregular and unsatisfactory printed results.

I have found that these undesirable results are due to the fact that the usually employed albumen, or gelatin, bichromate emulsions do not sufficiently penetrate the interstices of the rough plate and hence are easily detached therefrom by the further operations, or by the printing processes.

I have found that this objectionable feature may be overcome by employing acetic acid, or lactic acid, in the developing bath, particularly when gum arabic is used in the emulsion.

This valuable attribute can be further enhanced if benzine be added to the color ink and if a soft resin, such as elemi, or copal be employed.

As an example of one method of applying my process, I give the following:

The carefully cleaned and dried zinc plate is evenly and thoroughly covered with an emulsion consisting of 1 part best gum arabic dissolved in 3.5 parts water together with 10 parts ammonium bichromate dissolved in a small quantity of warm water. If desired, 10 parts alum may be added. The plate is then quickly dried and retained in a semi-dark room.

The plate is exposed under a positive in any suitable manner, the time of exposure

depending upon the intensity of the light and the depth of the positive.

The plate is now uniformly and completely treated with a developer consisting of 900 parts chemically pure glycerine, 50 parts water and 50 parts acetic acid, or lactic acid, which is thoroughly rubbed into the emulsion by means of a felt, or plush, cushion.

When the impression, or print, appears distinctly, the superfluous developer is removed by means of a rubber squeegee.

The color tincture composed of 900 c. c. denatured alcohol, 50 grams elemi, or copal, 27 grams shellac and 3 c. c. benzine, is then rubbed over the plate by means of a cloth and the fatty ink is then applied to the plate by means of a cloth until the impression appears in full black line. Defective places are immediately recognizable and can be remedied by intensive rubbing or additional developing.

Should the plate become too dry, developer must be again applied so that the emulsion is again saturated.

The plate is then placed in hydrochloric acid 1:25 which causes the bichromate film to dissolve.

The plate is now cleaned, etched in the usual manner and made ready for printing.

The lines on the plate thus produced are clear, clean, prominent and permanent.

By "bichromate emulsions" in my specification and claims I mean emulsions of bichromate and gum arabic, with or without, the addition of alum and by "organic developing acids" I mean acetic acid and lactic acid.

I do not limit myself to the particular times, temperatures, amounts or chemicals, or to the particular steps described in the above example, which are given simply as a means for clearly describing my invention.

What I claim is:

1. In the production of light-exposed bichromate gum emulsions upon zinc, the step which comprises the treatment of the exposed plate with a developer containing lactic acid and glycerine.

2. The process of producing zinc etched reproductions which comprises treating the zinc plate with a gum-arabic-bichromate emulsion, developing with a developer containing an organic developer acid, treating with a color tincture and a fatty ink, treat-

ing with hydrochloric acid and acid etching the resulting plate.

3. The process of producing zinc etched reproductions which comprises treating the 5 zinc plate with a gum-arabic-bichromate emulsion, developing with a developer containing an organic developer acid and glycerine, treating with a mixture containing a soft resin and a fatty ink, treating with hydrochloric acid and acid etching the resulting plate.

4. The process of producing zinc etched reproductions which comprises treating the 15 zinc plate with a gum-arabic-bichromate emulsion, developing with a developer containing lactic acid, treating with a mixture containing elemi and a fatty ink, treating with hydrochloric acid and acid etching the resulting plate.

5. The process of producing zinc etched 20 reproductions which comprises treating the zinc plate with a gum-arabic-bichromate emulsion, developing with a developer containing lactic acid, treating with a mixture containing a soft resin and a fatty ink, 25 treating with hydrochloric acid and acid etching the resulting plate.

6. The process of producing zinc etched reproductions which comprises treating the

zinc plate with a gum-arabic-bichromate emulsion, developing with a developer containing an organic developer acid and glycerine, 30 treating with a mixture containing a soft resin and a fatty ink, treating with hydrochloric acid and acid etching the resulting plate.

7. The process of producing zinc etched reproductions which comprises treating the zinc plate with a gum-arabic-bichromate emulsion, developing with a developer containing an organic developer acid, 35 treating with a mixture containing alcohol, benzine, shellac, a resin and a fatty ink, treating with hydrochloric acid and acid etching the resulting plate.

8. The process of producing zinc etched reproductions which comprises treating the zinc plate with a gum-arabic-bichromate emulsion, developing with a developer containing an organic developer acid and glycerine, 40 treating with a mixture containing alcohol, benzine, shellac, a resin and a fatty ink, 45 treating with hydrochloric acid and acid etching the resulting plate.

Signed at Berlin, Germany, this 25th day of May, 1923.

ANNA SCHWARZ, geb. HOPPEHEL.